

Sept. 28, 1937.

F. H. LEE

2,094,104

ART OF HAT MANUFACTURE

Filed Nov. 7, 1936

*Fig. 1*



*Fig. 2*



*Fig. 3*



*Fig. 4*



Inventor

FRANK H. LEE

*Blair & McLean, Inc.*  
Attorneys

## UNITED STATES PATENT OFFICE

2,094,104

## ART OF HAT MANUFACTURE

Frank H. Lee, Danbury, Conn.; Mary Josephine Fay Lee, Frank H. Lee, Jr., and The City National Bank and Trust Company, all of Danbury, Conn., executors of Frank H. Lee, deceased

Application November 7, 1936, Serial No. 109,782

## 3 Claims. (Cl. 2-175)

This invention relates to the art of hat manufacture and in its more specific aspects pertains to a method of finishing fur or felt hats and to the resulting hat article.

Among the objects of the present invention may be noted the provision of a novel method of treating fur or felt hats whereby to impart thereto a distinctive and unique finish; the provision of a novel and improved method of finishing hats; the provision of a method of finishing hats during their course of manufacture, which is simple and relatively inexpensive in practice; the provision of a hat having a distinctive and improved appearance; and the provision of a hat having a finish of such nature making it particularly acceptable for sports wear, although not limited thereto.

Other objects will be in part obvious and in part hereinafter pointed out in connection with the following analysis of this invention wherein is illustrated an embodiment of the invention in detail.

In the drawing—

Fig. 1 is a view of a hat article finished in accordance with the practice of the method of the present invention;

Fig. 2 is an enlarged partial section through the felt body of a hat at a partial stage in the finishing thereof in accordance with the present invention;

Fig. 3 is an enlarged partial section through the felt body of the hat following completion of the finishing operation in accordance with the present invention; and

Fig. 4 is a surface view of a portion of a hat as in Fig. 3.

In the practice of the method of the present invention, the hat body is fabricated in the rough by conventional or approved practices; that is to say, the hat bat is formed in the well known manner and is thereupon felted and shrunk down to body size, after which it is stretched and blocked, the hat at this stage of its manufacture being known to the trade as a "rough" hat. In the conventional manufacture of hats, such rough hat is generally "pounded" prior to finishing, the pounding operation consisting generally in subjecting the hat while rotating at high speed to the action of an abrasive sheet or its equivalent, thus to cut away from the body of felt the projecting surface fibers characteristic of a rough hat body prior to pouncing.

According to the method of the present invention, I eliminate the step of pouncing and hence the hat going to the finishing operations to be

described may be termed an "unpounded rough hat."

Such unpounded rough hat, according to the present invention, is put on a block of appropriate head size, and its surface fibers are scratched up in known manner. Such scratching up operation may consist of treatment of the hat surface with a wire brush or equivalent, with the result that the loose or projecting ends of the fur fibers are raised from the body of the felt.

Preferably, the crown and brim of the hat are now ironed, such ironing operation at this stage of manufacture causing the relatively long and projecting surface fibers to be uniformly laid, and also causing such fibers to be softened due to the heat imparted by the iron.

The hat is again subjected to a scratching up operation, as aforesaid, causing the laid and softened fibers to be again raised from the body of the felt as a preliminary to the clipping operation. Such clipping operation comprises generally the cutting or clipping away of the long ends of the raised fibers as by rotating knives or blades, the resulting hat having a surface characterized by relatively short fibers of uniform length projecting or raised from the body of the felt, the length of the fibers being long, however, in comparison to the surface fiber length of the hats subjected to the conventional pouncing step, and the hat consequently having a "rough" finish or appearance.

The clipped hat, while still on the block, as aforesaid, is next flanged, the flanging operation giving to the brim its "set" or flange, and the hat now possesses its final shape.

The flanged hat is thereupon subjected to the final finishing step, such comprising the surface treatment of the hat with a substance having adhesive properties, which, when worked in between the raised surface fibers as aforesaid causes adjacent fibers to group or bunch together and the relatively outer ends of the fibers of the bunches to become twisted and to knot together, with the substance as aforesaid then functioning to maintain adhesively the fibers in their twisted relation. By so working a substantial surface of the hat, there results a multiplicity of fiber groups or bunches of relatively short length and slightly spaced from each other throughout the treated area, it being understood that this treatment may be given to a particular surface, such as the crown, or to the entire surface of the hat.

The resulting hat has a finish or appearance somewhat resembling that of chinchilla, which

by reason of the set and interconnection of the fibers of the multiplicity of fiber bunches obtains throughout the life of the hat.

One substance having the desired adhesive properties which I have found to be satisfactory in causing adjacent fibers to "bunch", is gum tragacanth, although other natural gums, such as gum arabic, gum senegal, agar-agar, or artificial gums, such as ester gum, may be utilized to advantage. The gum tragacanth is applied sparingly over the surface of the hat as by a sponge or equivalent applying means and may be worked in between the surface fibers of the hat with the hand by the finisher, who will preferably wear a rubber glove. Preferably also, the gum is worked in with a circular motion and by the heel of the hand. It will be understood that methods of applying and working in the gum other than those suggested above may be practiced within the scope of the present invention.

Following the finishing operation as aforesaid the hat is trimmed and bound in the usual manner.

In the drawings, Fig. 1 represents a hat finished in accordance with the foregoing method, the hat illustrated being a man's hat comprising a crown 10 and a brim 11. It will be understood that such a hat configuration or contour as illustrated is typical only, as the invention is equally applicable to the finishing of women's fur or felt hats and head coverings generally.

In Fig. 2 is shown an enlarged portion of the felt body of a hat following the final clipping operation as aforesaid and prior to the final finishing operation. Reference character 15 designates the body of the felt formed of interfelts and interlocked fur fibers, the surface fibers 16 of which have been scratched up whereby they are raised from the body 15 of the felt and extend relatively outwardly therefrom. By reason of the clipping operation as aforesaid the raised fibers 16 are of substantially uniform length.

Referring to Figs. 3 and 4, such being representative of the relation of the surface fibers following the final finishing step, it will be noted that a plurality of adjacent fibers have been worked to form a multiplicity of slightly spaced fiber bunches 17, the fibers of which are twisted together so as to be interconnected adjacent their relatively outer ends.

The finished hat article as indicated in Fig. 1 possesses a unique and distinctive appearance 10 and has a surface texture which is soft and pleasing.

As many changes could be made in carrying out the above method without departing from the scope of the invention, it is intended that all 15 matter contained in the foregoing description shall be interpreted as illustrative and not in a limiting sense.

I claim:

1. A hat having a felt body and a surface finish 20 constituted by surface fibers of substantially uniform length extending from the body, the fibers being arranged in a multiplicity of spaced groups, and the fibers of a group being adhesively secured together adjacent their outer ends.

2. A hat having a felt body and a surface finish constituted by surface fibers of substantially uniform length extending from the body, the fibers being arranged in a multiplicity of spaced groups, the fibers of a group being twisted together adjacent their ends and adhesively maintained in such twisted relation.

3. A hat having a felt body and a surface finish constituted by surface fibers of substantially uniform length extending from the body, the fibers throughout the greater surface area of the felt body being arranged in a multiplicity of minutely spaced groups, the fibers of the groups being twisted together, at least some of the fibers of the groups carrying a substance operative adhesively 40 to maintain the fibers in such twisted relation.

FRANK H. LEE.